

1

3,019,081

## STABILIZED NITRIC ACID

Richard C. Doss and Jennings P. Blackwell, Bartlesville, Okla., assignors to Phillips Petroleum Company, a corporation of Delaware

No Drawing. Filed July 17, 1959, Ser. No. 827,975

12 Claims. (Cl. 23—157)

This invention relates to stabilized nitric acid. In one aspect this invention relates to the stabilization of concentrated nitric acid. In another aspect this invention relates to a stabilized oxidizer mixture comprising nitric acid and a quaternary ammonium compound.

Concentrated nitric acids such as are sold in the form of ordinary concentrated acid, white fuming nitric acid (WFNA), red fuming nitric acid (RFNA), and anhydrous nitric acid are important commercial products. These materials have many important uses such as for the preparation of fertilizers, in cleaning and etching solutions, etc. In recent years said concentrated nitric acids have been used as oxidizer ingredients for rocket propellants, in both bipropellant applications and in monopropellant applications. When used as the oxidizer component in a bipropellant system the acid is carried in the rocket or missile in a separate compartment or tank and is injected into the combustion chamber of the rocket motor as a separate stream where it contacts the fuel component, also injected as a separate stream. Said fuel component can be a hypergolic fuel, such as aniline, in which case spontaneous ignition takes place upon contact between the acid and the hypergolic fuel. Said fuel can also be a non-hypergolic fuel in which case the mixture formed when the acid and fuel are contacted is ignited by any suitable means such as a spark igniter. Monopropellant compositions consisting essentially of a fuel component such as an amine nitrate dissolved in nitric acid represent another application for said acids. In this type of application the monopropellant is stored in a tank carried by the rocket and is injected into the combustion chamber of said rocket where it is ignited.

Nitric acids, particularly concentrated nitric acids are not stable during storage, and tend to decompose according to the reaction:



Such decomposition of nitric acid during storage not only decreases the oxidizing power of the acid but also builds up pressure in the storage vessel. Over a period of time gas pressure can build up in the storage vessel to a point which constitutes a serious hazard, and can sometimes even result in rupture of the storage vessel. Even when the acid is stored in a vented vessel so that storage pressure is of no concern, the loss in product quality which occurs upon prolonged storage is serious. Thus, it is important for all uses of nitric acid that, if possible, said acid be stabilized to reduce decomposition during storage. Stabilization is particularly important where the acid must be stored in closed containers, such as in the fuel tanks in a rocket motor, etc.

We have discovered that quaternary ammonium compounds are effective stabilizers for nitric acid. Thus, broadly speaking, the present invention resides in a stabilized nitric acid containing a small but effective amount of a quaternary ammonium compound.

An object of this invention is to provide a stabilized nitric acid. Another object of this invention is to provide an improved oxidizer mixture which is suitable for use in reaction motors, such as rocket motors, etc. Still another object of this invention is to provide a stabilized nitric acid which can be safely stored in closed containers. Other aspects, objects, and advantages of the invention will

2

be apparent to those skilled in the art in view of this disclosure.

Thus, according to the invention, there is provided a stabilized nitric acid consisting essentially of nitric acid and from about 0.1 to about 10 weight percent of at least one quaternary ammonium compound characterized by a formula selected from the group consisting of



III



IV

25 wherein: each R is selected from the group consisting of alkyl, cycloalkyl, alkenyl, and cycloalkenyl radicals containing from 1 to 8 carbon atoms wherein when more than one carbon atom is present the carbon atom attached to the quaternary nitrogen atom is attached to adjoining carbon atoms by single valence bonds, and said radicals substituted with a substituent selected from the group consisting of nitro, nitrato, and cyano radicals, the total number of said substituents in said R groups being not greater than one-half the total number of carbon atoms in said R groups; R' is selected from the group consisting of alkylene radicals containing from 1 to 12 carbon atoms, and alkenylene radicals containing from 4 to 12 carbon atoms wherein the carbon atom attached to the quaternary nitrogen atom is attached to adjoining carbon atoms by single valence bonds; X is an anion selected from the group consisting of nitrate, perchlorate, monohydrogen phosphate, dihydrogen phosphate, hydrogen sulfate, sulfate, hydroxyl, orthoborate, dihydrogen borate, and tetraborate anions; a and b are each integers of from 1 to 4, and the product of a multiplied by the number of quaternary nitrogen atoms is equal to the product of b multiplied by the valence of said anion X.

30 It is to be noted that the compounds used in the practice of the invention are quaternary ammonium compounds as distinguished from acid salts of amines. The two classes of compounds are distinctly different chemically. As used herein and in the claims the term "quaternary ammonium compound" refers to a compound containing at least one nuclear nitrogen atom having its five so-called valence bonds attached to atoms (or radicals) other than a hydrogen atom. For example, such as four nitrogen to carbon bonds and one nitrogen to nitrate (or other anionic radical) bond. In other words, the available valence bonds of said nuclear nitrogen atom are satisfied by other than a hydrogen radical. For example, consider the two compounds (1) trimethylamine nitrate and (2) tetramethyl ammonium nitrate which have the formulas  $(\text{CH}_3)_3\text{NHNO}_3$  and  $(\text{CH}_3)_4\text{NNO}_3$ , respectively. It will be noted that in the acid salt trimethylamine nitrate one of the valence bonds of the nuclear nitrogen atom is satisfied by a hydrogen atom whereas in the quaternary ammonium compound tetramethyl ammonium nitrate all five valence bonds are satisfied by radicals other than hydrogen.

35 40 45 50 55 60 65 70 75 The two classes of compounds can also be distinguished by their reaction with strong bases. For example, when an acid salt such as trimethylamine nitrate is reacted with

sodium hydroxide the amine is liberated along with the formation of sodium nitrate and water; whereas a quaternary ammonium compound such as tetramethyl ammonium nitrate has no hydrogen available for the formation of water and there is obtained the tetramethyl ammonium hydroxide  $[(CH_3)_4NOH]$  and sodium nitrate, and no free amine is liberated.

Examples of quaternary ammonium compounds suitable for use in the practice of the invention include, among others, the following:

Tetramethylammonium nitrate  
Tetramethylammonium perchlorate  
Tetramethylammonium hydrogen sulfate  
Tetraethylammonium nitrate  
Triethylmethylammonium hydrogen sulfate  
Triethylmethylammonium nitrate  
Triethylmethylammonium perchlorate  
Triethylmethylammonium dihydrogenphosphate  
Diethyldimethylammonium nitrate  
Ethyltrimethylammonium nitrate  
Diallyldimethylammonium nitrate  
Tetra-n-propylammonium nitrate  
Tetra-n-propylammonium dihydrogen phosphate  
Tetra-n-propylammonium hydrogen sulfate  
Di(2-methylhexyl)dimethylammonium perchlorate  
Tetra-n-butylammonium nitrate  
Tetra-n-butylammonium perchlorate  
Trimethylpentylammonium perchlorate  
Ethyltripentylammonium perchlorate  
Dihexyldi-n-propylammonium nitrate  
Ethyltri-n-octylammonium nitrate  
Tetra-n-octylammonium nitrate  
Methyltri-n-octylammonium nitrate  
Methyltri-tert-octylammonium nitrate  
N,N,N',N'-tetramethyl diethylenediammonium di  
N,N,N',N'-tetra-n-butyl diethylenediammonium di  
Trimethylcyclohexylammonium nitrate  
Trimethylcyclohexylammonium metaborate  
Allyltrimethylammonium nitrate  
Triethyl-2-methallylammonium nitrate  
3-hexenyltriethylammonium nitrate  
Di-3-hexenyldimethylammonium nitrate  
Ethylidimethyl-2-cyclooctenylammonium nitrate  
Allyldiethylcyclohexylammonium perchlorate  
N,N,N,N',N',N'-hexamethyl methanediammonium  
trate  
N,N,N,N',N',N'-hexamethyl methanediammonium  
chlorate  
N,N,N,N',N',N'-hexaethyl methanediammonium  
chlorate  
N,N,N,N',N',N'-hexamethylethane-1,2-diammonium  
trate  
N,N,N,N',N',N'-hexamethylpropane-1,3-diammonium  
nitrate  
N,N,N,N',N',N'-hexamethylbutane-1,4-diammonium  
trate  
N,N,N,N',N',N'-hexamethylbutane-1,4-diammonium  
perchlorate  
N,N,N,N',N',N' - hexamethylbutane-14-bis(diam  
hydrogen phosphate)  
N,N,N,N',N',N' - hexamethylbutane - 1,4 - bis(amm  
hydrogen sulfate)  
N,N,N,N',N',N'-hexa-n-propylbutane1,4-diammonium  
nitrate  
N,N,N,N',N',N'-hexamethyloctane-1,8-diammonium  
trate  
N,N,N,N',N',N' - hexamethyldodecane-1,12-diam  
dinitrate  
N,N,N,N',N',N'-hexa(2 - nitroethyl)propane-1,  
monium dinitrate  
N,N,N,N',N',N'-hexa(2 - cyanoethyl)hexane-1,6-d  
ium dinitrate  
N,N,N,N',N',N'-hexa(2 - cyanoethyl)hexane-1,4-d  
ium dinitrate

N,N,N,N',N',N'-hexamethyl(2 - butene)-1,4-diammonium dinitrate  
 N,N'-dimethyltriethylene diammonium dinitrate  
 N,N'-dimethyltriethylene diammonium diperchlorate  
 N,N'-diethyltriethylene diammonium dinitrate  
 N-ethyl-N'-methyltriethylene diammonium dinitrate  
 N,N'-diisopropyltriethylene diammonium dinitrate  
 N,N'-dicyclohexyltriethylene diammonium dinitrate  
 N,N,N,N',N',N'-hexamethyl(4 - dodecene)-1,12-diammonium dinitrate  
 N,N,N,N',N',N'-hexaethyl(2,7 - diethyl-4-octene)-1,7-diammonium dinitrate  
 Tetramethyl ammonium tetraborate  
 Ethyltrimethyl ammonium orthoborate  
 Triethylmethyl ammonium perborate  
 Tetramethylammonium hydroxide  
 Tetraethylammonium hydroxide  
 Tetra-n-propylammonium hydroxide  
 Trimethylpentylammonium hydroxide  
 Methyltri-n-octylammonium hydroxide  
 N,N,N,N',N',N'-hexamethylmethane diammonium hydroxide  
 N,N,N,N',N',N' - hexaethyloctane - 1,8 - diammonium hydroxide

The quaternary ammonium compounds used in the practice of the invention can be prepared by any of a number of suitable methods well known to those skilled in the art. A first method comprises in general, the addition of a suitable alkyl chloride to a suitable amine which has been dissolved in a highly polar solvent such as nitrobenzene. The choice of the alkyl chloride, the amine, and the specific reaction temperature and quantities of reactants and solvents will of course depend upon the particular compounds it is desired to prepare as will be understood by those skilled in the art. Methyl alcohol can be used as a co-solvent to increase the solubility of the alkyl chloride in the polar solvent, if desired. After reaction of said alkyl chloride and said amine, the resulting quaternary ammonium chloride is separated and dried under vacuum. Said quaternary ammonium chloride is then dissolved in methyl alcohol and the exact percent of the chloride salt in solution is determined gravimetrically by means of silver chloride precipitation.

The thus obtained standardized alcoholic quaternary ammonium chloride solution is then treated with a stoichiometric amount of standardized alcoholic potassium hydroxide solution and the resulting potassium chloride which precipitates (essentially quantitative) is filtered. The filtrate is then treated with approximately a 10% excess of the acid corresponding to the quaternary ammonium salt to be prepared, e.g., nitric acid for nitrates, perchloric acid for perchlorates, etc. After the acid addition is complete, the mixture is evaporated to near dryness on a steam bath. The mushy residue is then dissolved in a minimum amount of isopropyl alcohol and the quaternary ammonium salt precipitates as a white crystalline product upon the addition of ethyl ether. The precipitated quaternary ammonium salt is filtered, washed with more ether and dried in a vacuum desiccator. This procedure has been found reliable and the quaternary ammonium salts so prepared are normally obtained in yields of 90-95 weight percent.

A second method comprises treating trialkylamine with a solution of an alkyl nitrate in ethyl ether and allowing the mixture to stand for several days, after which the solvent is evaporated.

A third method comprises treating a suitable amine with a suitable alkyl halide and then reacting silver nitrate with the resulting quaternary ammonium halide to produce the corresponding quaternary ammonium nitrate. Tetramethylammonium nitrate was prepared by this method.

The quaternary ammonium compounds are effective as stabilizers for nitric acids when used in small amounts

Generally, the amount used to stabilize the nitric acid is in the range of 0.1 to 10 percent, preferably within the range of about 0.5 to 5 percent, by weight of the total solution. The invention is applicable for stabilizing nitric acid of any concentration ranging from dilute acids containing as little as 1 weight percent  $\text{HNO}_3$  up to and including anhydrous acids containing essentially 100 weight percent  $\text{HNO}_3$ . However, since the more concentrated acids are more unstable, the invention finds its greatest use in stabilizing the more concentrated acids, particularly those containing at least about 50 weight percent, or more,  $\text{HNO}_3$ . The invention is particularly applicable for stabilizing the concentrated white fuming nitric acids, red fuming nitric acids, and anhydrous nitric acid which are available commercially. White fuming nitric acid usually contains about 90 to 99 weight percent  $\text{HNO}_2$ , from 0 to 2 weight percent  $\text{NO}_2$ , and up to about 10 weight percent water. Red fuming usually contains about 70 to 90 weight percent  $\text{HNO}_3$ , from 2 to 25 weight percent  $\text{NO}_2$ , and up to about 10 weight percent water. Fuming nitric acids, both white and red, having concentrations of water,  $\text{NO}_2$  and  $\text{HNO}_3$  different from those given can of course be stabilized in accordance with the invention.

In the practice of the invention the acid to be stabilized can be mixed with one or more of the above-described quaternary ammonium compounds in any convenient manner. It is generally preferred to add the quaternary ammonium compound to the acid at temperatures below about 50° C., e.g., 0 to 30° C., with good agitation. The resulting acid solutions have an enhanced stability as measured, for example, by measuring changes in pressure in a closed container containing the acid solutions in storage.

The following example will serve to further illustrate the invention.

*Example*

Anhydrous nitric acid was prepared by distilling red fuming nitric acid in the presence of sulfuric acid. Analyses of typical batches of a distilled anhydrous nitric acid showed that the product contained more than 99.8 weight percent  $\text{HNO}_3$  and less than 0.2 weight percent oxides of nitrogen.

The effectiveness of the quaternary ammonium compounds as stabilizing agents for nitric acid is shown by a comparison of the storage stability at 200° F. of a sample (9.9 grams) of said stabilized acid containing 0.1 gram of tetramethyl ammonium nitrate with another sample of anhydrous nitric acid containing no stabilizing agent. The thermal stability of said two samples was determined according to the following procedure.

A small glass tube constructed from one-fourth inch I.D. glass pipe, which will withstand a pressure greater than 1,000 p.s.i., is filled about two-thirds full (about 6 milliliters) with the nitric acid to be tested. Said tube is fitted with a safety head containing a blowout disc which will rupture at about 200 p.s.i. pressure. The small glass bomb is then placed in a constant temperature bath containing cold water and is connected to a pressure recorder and to a supply of compressed nitrogen gas. The pressure in said bomb is then increased to about 75 p.s.i.g. with nitrogen to check the system for leaks and, after checking, the pressure in said bomb is reduced to 20 p.s.i.g. The temperature in the constant temperature bath, which can be regulated to maintain a temperature of 200° F., is increased and the time at which a temperature of 200° F. is reached is taken as the start of the test. The test is terminated when the pressure in said bomb exceeds 100 p.s.i., or when the blowout disc is ruptured (the pressure rise is often rapid after 100 p.s.i. is reached). The storage life of the acid being tested is recorded as the time necessary for the pressure in said bomb to increase from 20 to 100 p.s.i. at a temperature of 200° F.

The results of the above tests showed that the pressure in the bomb containing the acid stabilized with tetramethyl ammonium nitrate increased slowly to 75 p.s.i.g. during the first 15 hours of the test and then decreased slowly to 33 p.s.i.g. during the succeeding 454 hours after which the test was terminated. Thus the stabilized acid had a storage life greater than 469 hours. The pressure in the bomb containing the sample of unstabilized nitric acid increased to 61 p.s.i.g. in 9 hours and the test was terminated at 28 hours when the pressure in said bomb had reached 100 p.s.i.g. Thus, the unstabilized acid had a storage life of only 28 hours.

The above tests show that the nitric acid stabilized with tetramethyl ammonium nitrate had a storage life more than sixteen times longer than the unstabilized nitric acid.

Since many possible embodiments can be made of this invention without departing from the scope thereof, it is to be understood that all matter herein set forth is to be interpreted as illustrative and not in a limiting sense.

We claim:

1. A stabilized nitric acid consisting essentially of nitric acid and from about 0.1 to about 10 weight percent of at least one quaternary ammonium compound characterized by a formula selected from the group consisting of



and

wherein: each R is selected from the group consisting of alkyl, cycloalkyl, alkenyl, and cycloalkenyl radicals containing from 1 to 8 carbon atoms wherein when more than one carbon atom is present the carbon atom attached to the quaternary nitrogen atom is attached to adjoining carbon atoms by single valence bonds, and said radicals substituted with a substituent selected from the group consisting of nitro, nitrato, and cyano radicals, the total number of said substituents in said R groups being not greater than one-half the total number of carbon atoms in said R groups; R' is selected from the group consisting of alkylene radicals containing from 1 to 12 carbon atoms, and alkenylene radicals containing from 4 to 12 carbon atoms wherein the carbon atom attached to the quaternary nitrogen atom is attached to adjoining carbon atoms by single valence bonds; X is an anion selected from the group consisting of nitrate, perchlorate, mono-hydrogen phosphate, dihydrogen phosphate, hydrogen sulfate, sulfate, hydroxyl, orthoborate, dihydrogen borate, and tetraborate anions; a and b are each integers of from 1 to 4, and the product of a multiplied by the number of quaternary nitrogen atoms is equal to the product of b multiplied by the valence of said anion X.

2. A stabilized nitric acid according to claim 1 wherein the nitric acid to be stabilized contains at least 50 weight percent  $\text{HNO}_3$ .

3. A stabilized nitric acid according to claim 1 wherein the nitric acid to be stabilized contains at least 70 weight percent  $\text{HNO}_3$ .

4. A stabilized nitric acid according to claim 2 wherein the amount of said quaternary ammonium compound is within the range of about 0.5 to 5 weight percent.

5. A stabilized nitric acid according to claim 3 wherein

the amount of said quaternary ammonium is within the range of 0.5 to about 5 weight percent.

6. The stabilized nitric acid of claim 1 wherein said quaternary ammonium compound is N,N'-dimethyltriethylenediammonium dinitrate.

7. The stabilized nitric acid of claim 1 wherein said quaternary ammonium compound is N,N'-diethyltriethylenediammonium dinitrate.

8. The stabilized nitric acid of claim 1 wherein said quaternary ammonium compound is N-ethyl-N'-methyltriethylenediammonium dinitrate.

9. The stabilized nitric acid of claim 1 wherein said quaternary ammonium compound is tetramethylammonium nitrate.

10

10. The stabilized nitric acid of claim 1 wherein said quaternary ammonium compound is tetraethylammonium nitrate.

11. The stabilized nitric acid of claim 1 wherein said quaternary ammonium compound is N,N,N,N',N',N'-hexamethylpropane-1,3-ammonium dinitrate.

12. The stabilized nitric acid of claim 1 wherein said quaternary ammonium compound is N,N,N,N',N',N'-hexamethylbutane-1,3-ammonium dinitrate.

References Cited in the file of this patent

UNITED STATES PATENTS

2,037,762 Cole \_\_\_\_\_ Apr. 21, 1936  
2,814,593 Beiswanger \_\_\_\_\_ Nov. 26, 1951